

## COMBUSTION PROCESS

Warren C. Simpson, Berkeley, Calif., assignor to Shell Development Company, New York, N.Y., a corporation of Delaware

No Drawing. Application February 25, 1957  
Serial No. 641,874

6 Claims. (Cl. 158—117.5)

The present invention relates to the operation of furnaces in which fluid fuels are burned. More particularly, it is concerned with a method of improving and controlling the radiant heat or emissivity of flames produced in furnaces.

In many types of furnaces wherein the fuel burned is oil, gas, or mixtures thereof, at least a part of the heat released by the flame is transferred from the flame to the body being heated by means of radiation. This either occurs directly, as in the case of a solid charge, or indirectly, as in the case of a liquid charge. Open hearth steel furnaces, lime and cement kilns, annealing furnaces, tube still heaters, cracking furnaces, and the like are examples of many types of furnaces largely dependent upon radiant heat transfer. The present invention is especially directed to the operation of open hearth furnaces in steel making processes, but the principles and process apply to these other types of furnaces as well.

In all of such types of furnaces, the proportion of heat transferred to the charge by radiation is largely fixed by the design of the furnace and by the characteristics of the flame. For example, in an open hearth furnace nearly all of the heat is transferred to the charge by radiation. In the usual case of a tube still heater or kiln to which the charge is continuously fed at a constant temperature and rate, the proportion of radiant heat transfer depends upon the ratio of the tube surface area which the flame "sees" to the tube surface area which is in contact with the combustion gases, but which the flame cannot "see." As long as outlet temperatures must remain constant at a predetermined value, which is almost always true, the heat absorption profile of the charge within the furnace has not heretofore been a variable, once a particular furnace design is selected and a particular fuel utilized.

Industrial furnaces are ordinarily extremely large capital investments and it is obvious that increased flexibility in the operation of such furnaces would be highly advantageous.

The addition of foreign bodies to fuel oils for the purpose of increasing emissivity of the flames during burning or combustion is successful but entails a number of serious disadvantages. One of these comprises the relatively high expense of suitable forms of carbon such as carbon black or acetylene black. The benefits of the reduction in the time necessary to heat a batch of steel in an open hearth furnace, and thereby the monetary savings effected, are cut substantially in half by the cost of the carbon black added to the fuel oil. A technical disadvantage comprises the extremely high viscosity of concentrates of the carbon black. One phenomenon which has been observed in the use of solid particulate materials such as carbon blacks comprises their agglomeration into chain-like structures, thus reducing their emissivity which is at a maximum when the particle is either spheroidal or spherical in shape.

It is an object of the present invention to provide a method of controlling the radiation effects within fur-

naces. It is a more particular object of this invention to provide increased flexibility in the radiation effects of flames burning in furnaces. It is a further object of the invention to improve the economic aspects of operating such furnaces. Other objects will appear hereinafter.

Now, in accordance with the present invention, it has been found that the radiation or emissivity (in the infrared spectral region) of a flame being burned in a furnace may be increased by precipitation of a substantial proportion of the components having molecular weights above about 1000 (preferably 1000-5000) present in a residual fuel oil to yield agglomerates greater than colloidal size and thereafter burning the fuel oil containing said particles, whereby flames of increased emissivity are obtained.

Residual fuel oils generally consist of a blend of vacuum flashed or thermally cracked residue in a mixture of lighter distillates (cutter stock) of relatively low viscosity. When the aromatic or heteroaromatic components of the residue having molecular weights greater than about 1000 are maintained in true solution by the lower molecular weight aromatics and heteroaromatics in the system, the fuel oil will be optically clear when examined in thin layers. When the solubilizing power of the lower molecular weight components of the fuel oil is not sufficient to maintain true solution, the occurrence of molecular association between various of the higher molecular weight polar components leads to the formation of loose aggregates of molecules into clusters which eventually grow into aggregates sufficiently large to be visible to the unaided eye as a precipitate. This imperfect solubilization of the high molecular weight components may be brought about by the addition of paraffinic components to the system.

In accordance with a preferred version of the present invention, the precipitated particles (including agglomerates or originally discrete particles) are distributed in particle size over a range from about 0.5 micron to about 150 microns, so that as the relatively smaller particles are consumed and disappear from the flame, the relatively larger particles still persist in acting as radiating bodies. In accordance with one phase of the present invention, this range in particle size of the precipitated particles may be effected by a differential time of particle size existence between several portions of the residual fuel being introduced into the furnace. If, for example, the smallest particles are formed by a residence time outside of the furnace and prior to burning of about 5 seconds or less, then it is preferred that an appreciable portion of the fuel oil be subjected to precipitation techniques for a time prior entrance into the furnace of at least about 30 seconds or more, so that the necessary time for particle growth is gained after which both particle-containing residual fuel streams are introduced, either together or separately, into the flame-burning area.

Since it is preferred that substantially continuous elevated emissivity throughout the entire area of the flame is obtained, it is preferred that at least about 10% by weight of the precipitated particles have diameters less than about 0.5 microns and at least 10% by weight of the particles have diameters greater than about 10 microns. Thus, there is virtual insurance that the flame will contain at all times an emission-improving portion of radiating particles, even though the flame be of a length from about several inches to as much as 35 feet. Flames from about 15 to 30 feet are commonly employed in such large scale industrial installations as open hearth steel furnaces and the like. The upper limit of particle size is determined as that size particle which will just be consumed in the particular flame whose length, temperature, percent excess air and linear

velocity are known. For any given flame and a knowledge of the furnace geometry this maximum particle size can be determined.

The fuel oils to be treated in accordance with the present invention are defined as being asphaltogenic in nature, by which is meant that said fuel oils are normally residual fuels or contain substantial quantities of residual petroleum components, said residual components comprising in part those bodies of reduced solubility characteristics which have molecular weights above about 1000, usually 1000-5000.

A further improvement in the present invention, especially as applied to situations such as exist in open hearth steel making furnaces, comprises maintaining the flame profile substantially constant during the entire steel making process, and varying the radiation of the flame by controlling the proportion of suitable particles in the fuel stream. A still further improvement in this respect comprises maintaining the total fuel input substantially constant throughout the steel making process, thus maintaining the flame profile substantially unaltered during the same period, but varying the radiation characteristics thereof by variation in particle proportion.

The open hearth furnace is a batch furnace. Steel scrap, pig iron, and sometimes a small proportion of ore are charged to the furnace, melted and refined. In the first stage of the melt, the "charging period," the solids are cold and present an irregular surface to the flame and combustion gases. The actual charge to the furnace is normally carried out in a series of steps since the unmelted mass usually is too large for the entire charge to be made at one time. Consequently, substantially half of the charge is inserted in the furnace and partially or fully melted before further portions of the charge are added. Upon commencement of heating at least a portion of the charge melts sufficiently to substantially submerge the remaining solids and the surface of the charge becomes flat. When this stage has been reached, the so-called "melting period" begins. When the ingredients have all reached the melt stage (or substantially so), the "refining period" starts, during which the liquid charge is maintained at a high and substantially constant temperature for the necessary time to complete purification by separation of the slag from the main body of the melted steel.

It is economically desirable to minimize the time consumed during the charging and melting periods in order to maintain a high rate of production of steel from the furnace. During these first two periods (charging and melting) the temperature is being raised continually and, consequently, during this time the maximum degree of radiation from the flame is desirable. The maximum fuel input rate is limited by the melting temperature of the roof of the furnace as well as the optimum flame profile for efficient transfer of heat from the flame to the melting charge. During the charging period high fuel input rates may be employed when both the charge and the furnace refractory roof are relatively cool. However, during the melting period, the fuel input rate is limited by the maximum allowable temperature of the refractory roof which is ordinarily in the order of 2800-3000° F. Since the temperature of the charge during this period gradually rises from 2400 to 2600° F., there is a very small margin between required and maximum allowable furnace temperatures.

While the fuel input rate can be varied, it will be obvious that the flame profile will alter radically with any change made in this input rate. Hence, it is desirable to establish the optimum flame profile for a given rate of fuel input and thereafter maintain the same rate of total fuel consumption. The present process is based upon these considerations and provides the flexibility necessary for successful operation thereof.

Fuels have been modified in the past by the incorporation of solid fuel materials, especially powdered coal.

However, the use of powdered coal in fuel oil suspension does not provide the desired increase in radiant heat, since the powdered coal particles are either relatively extremely coarse and consequently do not present the surface area necessary for optimum black body radiation, or (due to burning rates slower than that of oil) must be ground much finer than precipitated oil particles if they are to be completely consumed. Other solid fuel components used as proposed heretofore, have been incorporated in the entire body of the fuel oil and consequently permitted no latitude in the alteration of the radiation of the flame which must necessarily have remained at a constant value for any total rate of fuel input. Moreover, the principal disadvantage which was experienced with these prior art coal and carbon black suspensions comprised the difficulty of maintenance of the suspension, since in the relatively dilute form in which they are normally employed the particles are not self-supporting and tend to settle out. This property may be overcome in part by incorporation of certain suspending agents and surfactants, but this is an uneconomical means of creating and maintaining the suspensions and also entails certain problems such as the creation of undesirable ash. Since the fuel input into a large furnace such as an open hearth furnace is extremely high, the ash problem becomes serious due to deposition thereof on the sides of the furnace and the operating parts thereof.

The improvement caused by this invention is apparently based upon the increased emission of radiant energy at wave lengths at which solid matter absorbs most efficiently, i.e., in the infrared range.

The method of the present invention applies especially to those residual fuel oils having precipitation indices between 25 and 80, preferably between about 40 and about 65. These include especially straight run and cracked flasher bottoms as well as catalytically cracked gas oil bottoms as well as thermally and catalytically cracked reforming bottoms. The precipitation index is defined as the percentage of alpha-methyl naphthalene in a mixture with cetane which will just dissolve the least soluble component of the residue: the higher the precipitation index the more insoluble the residue.

The particles are precipitated in an amount between about 1 and about 10% by weight, based on the total fuel. This is preferably effected by addition to the asphaltogenic residual fuel oil of a precipitating liquid having a low solvency index, the latter term being defined as follows: The solvency index of a liquid is defined as the volume percentage of alpha-methyl naphthalene in an alpha-methyl naphthalene-cetane mixture equivalent in solvency to that of the liquid under examination. For the most part, low solvency precipitating liquids include paraffinic hydrocarbons having from 3 to 20 (preferably 5-20) carbon atoms per molecule, the most practical one of which is an extracted kerosene fraction, since this product contains a high concentration of the higher normal alkanes which are still liquid at ambient temperature. These higher normal alkanes, preferably having molecular weights between 150 and 250, are more effective precipitants than the lower alkanes.

Following are typical solvency indices for specific compounds:

| Compound:                | Solvency index |
|--------------------------|----------------|
| Alpha-methyl naphthalene | 100            |
| Toluene                  | 77             |
| Cyclohexane              | 47             |
| 1-octene                 | 20.8           |
| 1-dodecene               | 19.0           |
| n-Hexane                 | 18.2           |
| n-Octane                 | 16.7           |
| n-Dodecane               | 10.3           |
| n-Tetradecene            | 7.4            |
| n-Hexadecane             | 0.0            |

Other precipitating liquids include normally gaseous hydrocarbons, such as propane and butane, as well as the normally liquid hydrocarbons, such as hexane or decane.

The proportion of precipitating liquid to be added to the residual fuel oil will depend upon a number of factors, including the solvency index of the precipitating liquid, the precipitation index of the fuel oil, the proportion of particles desired, and the average diameter of the particles required, in addition to the lapse of time between mixing of the precipitant with the fuel oil and the time of combustion. Normally, however, it will be found that precipitants having from 3 to 20 carbon atoms per molecule and having a solvency index between about 0 and about 50 when added to the preferred type of residual fuel oils having precipitation index between about 20 and about 80 are utilized in amounts from about 20% to about 80% by weight, based on the fuel oil, and ordinarily then constitute not only a precipitating agent but also a combustible component of the fuel oil composition.

It has been ascertained that non-aromatic (aliphatic and/or cycloaliphatic) precipitating agents, such as kerosene and the like, actually exhibit a lower emissivity than the ordinary residual fuel oil. However, when the precipitating agent and the fuel oil are combined in such proportions as to precipitate particles as described above, the emissivity (in the infra red region) of the burning fuel composition is substantially higher than that experienced by either the fuel oil alone or by the precipitating agent alone.

The effect of increasing the emissivity of the combustible fuels is of great economic significance since it has been ascertained that the average time of completing a run in a standard commercial open hearth furnace can be reduced as much as about 10%.

The addition of the precipitating liquid to the residual fuel oil is preferably effected just prior to injection into the furnace and combustion of the fuel composition. The timing will be adjusted to produce the optimum size of particles in accordance with the limitations set forth hereinbefore but normally will be between about 1 second and 24 hours and preferably between about 30 seconds and  $\frac{1}{2}$  hour. The production of particles in a residual fuel, according to the present process, results in substantially spherical particles which, upon aging in the fuel oil composition, tend to agglomerate into larger bodies which still maintain their essentially spherical shape. This is sharply differentiated from the chain-like agglomerates which are created upon the aging of carbon black particles suspended in fuel oils.

In order to maintain a substantially constant supply of radiating precipitated bodies throughout the entire length of a fuel flame such as in an open hearth furnace, it is preferred that the particle size distribution be spread between the limits already stated, namely, between about 0.5 micron and about 150 microns. This may be difficult to attain if the precipitating agent is added to the fuel oil at only one particular time prior to combustion of the fuel oil composition. Therefore, in accordance with one phase of this invention, it is a preferred process to inject portions of the precipitating agent into fuel oil being fed to a burner at two or more time units prior to burning so that an elapsed time is permitted for part of the particles to agglomerate or grow and form the relatively coarser varieties which have a more extended life prior to being completely burnt in the flame during combustion. This multiple addition of a precipitating liquid added thereto so as to enable the growth or agglomeration of particles to occur. The two or more portions of the fuel may be combined at the burner or may be injected into the combustion area through separate nozzles. An aging opportunity can be created by passing that portion of the fuel oil in which the relatively larger particles are to be formed into a storage tank preferably containing agitation means or through a coil designed to increase the residence time of the fuel oil therein so as to provide

the necessary extended particle formation period prior to burning.

By utilization of the present process of precipitating fuel components in the fuel stream of such furnaces, it has been found that great economic advantages can be obtained, for example, in the cycle time for the production of steel. By the precipitation of 1.5-5% insoluble particles into the fuel oil utilized for the heating of an open hearth furnace, for example, during the charging and melting stages but omitted during the refining stage, a 10% reduction in total cycle time can be effected. By maintaining the total fuel input constant during the entire period of steel production (or during any other comparable process, such as cement production) the flame profile was substantially unaltered, but the radiation thereof was radically changed by the injection or omission of the colloidal particles. The increased flame luminosity did not appear to affect refractory life in such furnaces since the temperature of the flame was not substantially different from that of the flame without particle formation. The following examples illustrate the process of the present invention.

#### Example I

A fuel composition was prepared by the addition of 40 parts by weight of an extracted kerosene (having a solvency index of about 30) to 60 parts by weight of two fuel oils having the following properties:

|                                                | Fuel Oil A | Fuel Oil B |
|------------------------------------------------|------------|------------|
| Unblended thermal residue, percent             | 57         | 89.0       |
| Lube oil extract, percent                      | 18         | 0          |
| Thermally cracked pressure distillate, percent | 25         | 11.0       |
| Gravity, ° API                                 | 12.2       | 8.5        |
| Flash, Pensky-Martin, ° F                      | 218        | 194        |
| Viscosity, SSF, at 122° F                      | 27.5       | 164        |
| Pour point, ° F                                | -10        | +25        |
| Sulfur, percent                                | 0.93       | 0.89       |
| Precipitation index                            | 48         | 48         |

When these combinations of kerosene and fuel oils were burned after a particle formation period of 1-10 minutes and the flame examined for radiation by means of an infra red spectrometer, it was found that the combustion of the compositions containing the resulting precipitated particles gave a substantially greater intensity in a useful radiation range (1-3.5 microns) than are produced by combustion of the unmodified fuel oils.

The same was true after the composition containing the precipitating liquid and the resulting particles was allowed to age for 24 hours.

The deleanu extracted kerosene employed in this test had the following properties:

|                                 |         |
|---------------------------------|---------|
| Gravity, ° API                  | 42.5    |
| Solvency index                  | 30      |
| Aromatics, percent              | 3.7     |
| Boiling range, ° F              | 384-497 |
| Flash point, Pensky-Martin, ° F | 155     |

When the compositions containing the precipitating liquid have been aged for about 1 minute it can be suitably used in the heating of an open hearth steel furnace utilizing 90 pounds of air pressure for atomizing the total fuel charge. The total fuel including the residual fuel oil and the precipitating liquid is about 5 gallons per minute for the purpose of heating a total steel charge of about 76 tons. Parallel runs in the same steel open hearth steel furnace show that substantially shorter times (approximately by 10%) are necessary for reaching the correct stage of charging and melting of the steel charge when precipitated fuel particles are present in the fuel oil composition than when the unmodified fuel oils are employed.

Varying proportions of the above-described kerosene and fuel oil A were mixed to determine the amount of

7  
fuel precipitated in the form of particles. The table summarizes the results obtained:

| Percent (Vol.) Fuel Oil A | Percent (Vol.) Kerosene | Percent (Vol.) Fuel Oil A Precipitated |
|---------------------------|-------------------------|----------------------------------------|
| 65                        | 35                      | 4.3                                    |
| 60                        | 40                      | 8.3                                    |
| 55                        | 45                      | 9.5                                    |
| 50                        | 50                      | 9.6                                    |

I claim as my invention:

1. A method of improving the radiation emission of an asphaltogenic residual fuel oil having a precipitation index of at least 40 during the combustion thereof which comprises precipitating therein between about 1% and about 10% by weight, based on total fuel components, of high molecular weight fuel components as substantially spherical particles by admixing 20-80% by weight based on the fuel oil, of aliphatic hydrocarbons having 3-20 carbon atoms per molecule therewith and thereafter burning the particle-containing fuel, whereby its emission of radiant energy in the infra red range is increased, said admixing being effected from 30 seconds to one-half hour prior to combustion.

2. A method of improving the radiation emission of an asphaltogenic residual fuel oil having a precipitation index of at least 40 during the combustion thereof which comprises precipitating therein between about 1% and about 10% by weight, based on total fuel components of insoluble fuel substantially spherical particles by admixing 20-80% by weight, based on the fuel oil, of substantially aliphatic C<sub>3</sub>-C<sub>20</sub> hydrocarbons therewith and thereafter burning the particle-containing fuel, whereby its emission of radiant energy in the infra red range is increased, said admixing being effected from 30 seconds to one-half hour prior to combustion.

3. A method of improving the radiation emission of an asphaltogenic residual fuel oil having a precipitation index of at least 40 during the combustion thereof which comprises precipitating therein between about 1% and about 10% by weight, based on total fuel components, of insoluble fuel components substantially spherical particles having diameters between 0.5 microns and 150 microns by admixing 20-80% by weight, based on the fuel oil, of non-aromatic hydrocarbons boiling in the kerosene range and thereafter burning the particle-containing fuel, whereby its emission of radiant energy in the infra red

range is increased, said admixing being effected from 30 seconds to one-half hour prior to combustion.

4. A method of improving the radiation emission of an asphaltogenic residual fuel oil having a precipitation index of at least 40 during the combustion thereof which comprises precipitating therein between about 1% and about 10% by weight, based on total fuel components, of fuel component substantially spherical particles of substantially spherical shape, at least 80% by weight of which have diameters between about 0.5 micron and 150 microns and thereafter burning the particle-containing fuel, whereby its emission of radiant energy in the infra red range is increased, said precipitating being effected by addition to the fuel oil of 20-80% by weight based on the fuel oil of hydrocarbons having 3-20 carbon atoms per molecule at a time between about 1 second and 24 hours prior to combustion.

5. A method of improving the radiation emission of an asphaltogenic fuel oil having a precipitation index of 25-80 during the combustion thereof which comprises adding thereto, at a time between 1 second and 24 hours prior to combustion, 20-80% by weight, based on the fuel oil, of aliphatic hydrocarbons having 3-20 carbon atoms per molecule, whereby 1-10% by weight, based on the oil plus hydrocarbons, of components having molecular weights above about 1000 are precipitated as substantially spherical particles and thereafter burning the resulting mixture, the incandescent particles increasing emission of radiant energy in the infra-red range during burning.

6. A method of improving the radiation emission of an asphaltogenic fuel oil having a precipitation index of at least 25 during the combustion thereof which comprises adding thereto, at a time between 1 second and 24 hours prior to combustion, 20-80% by weight, based on fuel oil, of aliphatic hydrocarbons having 3-20 carbon atoms per molecule, whereby 1-10% by weight, based on the oil plus hydrocarbons, of components having molecular weights above about 1000 are precipitated as substantially spherical particles and thereafter burning the resulting mixture, the incandescent particles increasing emission of radiant energy in the infra-red range during burning.

References Cited in the file of this patent

UNITED STATES PATENTS

2,780,538 Chilton Feb. 5, 1957

FOREIGN PATENTS

340,314 Great Britain Dec. 29, 1930